

March 30, 1926.

G. A. MONTGOMERY

1,578,543

METHOD OF MAKING DEEP WELL AUGER STEMS

Filed August 8, 1924

Fig. 1.



Fig. 4.



Fig. 5.



Fig. 6. 21



Fig. 7. 21



Fig. 8.



Fig. 9. 27



Inventor,  
Gustavus A. Montgomery,  
by Geyer & Geyer  
Attorneys.

Patented Mar. 30, 1926.

1,578,543

# UNITED STATES PATENT OFFICE.

GUSTAVUS A. MONTGOMERY, OF TITUSVILLE, PENNSYLVANIA, ASSIGNOR TO TITUSVILLE FORGE COMPANY, OF TITUSVILLE, PENNSYLVANIA, A CORPORATION OF MARYLAND.

## METHOD OF MAKING DEEP-WELL AUGER STEMS.

Application filed August 8, 1924. Serial No. 730,796.

To all whom it may concern:

Be it known that I, GUSTAVUS A. MONTGOMERY, a citizen of Finland, and residing at Titusville, in the county of Crawford and State of Pennsylvania, have invented new and useful Improvements in Methods of Making Deep-Well Auger Stems, of which the following is a specification.

This invention relates generally to a method of making tools used in boring artesian and oil wells but more particularly to a method of making auger stems such as shown in United States Letters Patent No. 1,188,982, granted to L. E. Nebergall, June 27, 1916.

The chief object of the invention is the provision of a novel and efficient method of making auger stems of this character which will afford a marked saving in time, material and cost of manufacture over other methods heretofore employed.

Another object is to provide a method of forging spiral or auger stems in such a manner that the twisting or spiral formation of the stem-wings is performed from the same heat treatment as that initially given the stock or billet for shaping it into cruciform cross section with the wings straight and parallel with the axis of the stem.

In the accompanying drawings:

Figure 1 is a fragmentary side view of the auger or spiral stem made by my improved method. Figure 2 is a cross section thereof on line 2—2, Fig. 1. Figure 3 is a fragmentary front elevation of a well-known type of forging press used in practicing the invention and showing the first step of the method. Figures 4, 5 and 6 are end views of the forging dies showing the various stages in shaping the auger stem. Figure 7 is a side view of the dies illustrated in Figure 6. Figure 8 is an end view of the dies employed in the final or straightening step of the method.

Similar characters of reference indicate corresponding parts throughout the several views.

The auger or spiral stem made in accordance with the method constituting the subject matter of this application consists of a plurality of ribs or wings 10 which are disposed radially to the longitudinal axis of the stem and which are also inclined or twisted so as to extend helically about said

longitudinal axis. The pitch of the wings is relatively great and the length of the stem ordinarily used in practice ranges from twenty to forty feet. At its upper and lower ends, the spiral stem is provided with the usual necks or coupling collars containing the threaded boxes 11, 12, respectively.

In practicing my method for making the spiral stems any suitable and well-known forging press may be employed. That shown in the drawings by way of example, consists of columns 13, 13 on which the vertically movable press head 14 is guided. The numeral 15 indicates the anvil or bottom dies and 16 the upper dies carried by the press head. As shown in Figs. 3, 4 and 5, these dies are provided in their opposing faces with a series of longitudinal recesses or cavities 17, 18 extending from end to end thereof. These cavities are of the desired shape in cross section to produce by stages the radial wings 10 of the stem. Another forging press located alongside the one just described contains upper and lower dies 19 and 20, respectively, which are likewise provided in their opposing faces with longitudinal recesses or cavities 21 extending from end to end thereof. As illustrated in Figs. 6 and 7, the opposing faces of these dies are curved in the manner shown at 22 to produce the twisted or spiral form of the wings. The curved surfaces of said dies, on one side of the longitudinal axis thereof, are inclined in one direction while the corresponding surfaces on the other side of such axis are inclined in the opposite direction in accordance with the direction of spirality of the stem-wings on diametrically opposite sides of its axis.

After having sized the steel forging billet 23, from which the spiral stem is made, into substantially rectangular cross-section, it is placed diagonally between the straight faces of the dies 15, 16 for the purpose of squaring the corners 24 to the approximate width or thickness of the stem-wing 10 when finished. In this diagonal position, the billet is now placed over the cavity 17 of the lower die and the forging press is operated to work the billet into the cruciform shape shown in Fig. 4, the vertically-aligned wings being formed in the opposing die-cavities and the horizontally-aligned wings being formed between the opposing straight faces

of said dies on opposite sides of their cavities. The billet is then placed over the cavity 18 of the lower die and forged in like manner into the shape disclosed in Fig. 5. 5 This breaking down process completes the first step of providing the stem with the radial wings extending lengthwise thereof and parallel with its longitudinal axis. While only two sets of cavities have been 10 shown in the dies 15, 16, it is to be understood that any number may be employed to attain the desired results. In order to attain symmetry and uniformity of width and thickness of the several wings, the billet is 15 preferably given a quarter turn from time to time during the forging operation.

The next step in the method of making the auger stem is that of twisting the longitudinal wings formed in the first step into 20 twisted or helical form. The heat remaining from the breaking process is utilized in shaping the wings into spiral form, no further heating of the stem being necessary. While in such heated state, the billet is immediately forged between the dies 19 and 25 20, one set of diametrically-disposed wings being first shaped, as shown in Figs. 6 and 7, after which the other set is operated upon by simply giving the stem a quarter 30 of a turn. By this movement, the untwisted wings are removed from the cavities 21 and placed between the opposing curved faces 22 of the dies, while the finished or twisted wings occupy said cavities. The latter are 35 of sufficient width to accommodate a given length of the twisted wings.

By performing the twisting operation on the stem-wings immediately after the breaking down process, it not only eliminates re-heating of the stem but the latter is prevented from bending out of shape, inasmuch as the helical or twisted wings add stiffness to the stem and keep it straight.

In view of the great length (20 to 40 feet) 45 in which these spiral stems are made, it is necessary to forge them in sections. By preference, it is first forged at the center and then toward its opposite ends until the spiral guide wings are completely formed.

After thus forging the stem, it is placed 50 between a pair of straightening dies 25, 26, the lower die 25 containing a V-shaped groove or recess 27 upon which the lower spiral wings are seated. A fuller 28 is placed between the bottom face of the upper die 26 and in the groove formed between the opposing pairs of wings. By this arrangement a three-point bearing is provided 55 for the spiral stem, whereby it is effectually straightened in both lateral and vertical planes by the one operation.

The shaping dies are originally designed 60 for the largest stems made and should it be desired to make smaller stems of varying sizes, the die-cavities may be fitted with

suitable liners, thereby controlling the sizes wanted without taking measurements during the forging process.

The necks at the ends of the stems may be formed in any suitable and well known 70 manner.

This improved method of making spiral stems has proven very efficient and reliable in practice. Aside from affording a material saving in time and labor over methods 75 heretofore employed, this method reduces the cost of manufacture over 75% and results in a saving of material of approximately 50%. Furthermore, the stem is supported on all sides during the forging operation, rendering a more thorough and uniform working of the material and eliminating the formation of so-called "cold shuts."

I claim as my invention:—

1. The method of making a tool stem having radial wings extending lengthwise thereof, which consists in forging a billet of rectangular cross-section into a stem substantially cruciform in cross-section, positioning the resulting wings of the stem between dies shaped to twist one set of diametrically opposite wings helically about the longitudinal axis of the stem, and then rotating said stem to bring the other set of wings between said dies.

2. The method of making a tool stem having radial wings extending lengthwise thereof, which consists in forging a billet of rectangular cross-section into a stem substantially cruciform in cross-section, immediately positioning, without further heat treating, the resulting wings of the stem between dies shaped to twist one set of diametrically opposite wings helically about the longitudinal axis of the stem, and then rotating said stem a quarter of a turn to bring the other set of wings between said dies, said stem being fed longitudinally and intermittently after the two successive twisting operations of the dies.

3. The method of making a tool stem having radial wings extending lengthwise thereof, which consists in forging a steel billet into a stem substantially cruciform in cross-section, positioning the resulting wings of the stem between dies shaped to twist one set of diametrically opposite wings helically about the axis of the stem while the other set remains unchanged, and then rotating said stem to bring such other set of wings between said dies while the previously twisted wings are unacted upon, said stem being fed longitudinally through the dies only after two successive operations on the stem-wings, whereby portions of the stem from end to end thereof are successively acted upon to produce continuous and uninterrupted spiral wings thereon.